



US007293597B2

(12) **United States Patent**  
Parkos, Jr. et al.

(10) **Patent No.:** US 7,293,597 B2  
(45) **Date of Patent:** Nov. 13, 2007

(54) **NON-OXIDIZABLE COATING**

(75) Inventors: **Joseph J. Parkos, Jr.**, East Haddam, CT (US); **Gary M. Lomasney**, Glastonbury, CT (US); **Joshua E. Persky**, Carbondale, CO (US)

(73) Assignee: **United Technologies Corporation**, Hartford, CT (US)

(\*) Notice: Subject to any disclaimer, the term of this patent is extended or adjusted under 35 U.S.C. 154(b) by 11 days.

(21) Appl. No.: 11/526,965

(22) Filed: Sep. 26, 2006

(65) **Prior Publication Data**

US 2007/0017654 A1 Jan. 25, 2007

**Related U.S. Application Data**

(63) Continuation of application No. 10/973,132, filed on Oct. 26, 2004, now Pat. No. 7,207,373.

(51) **Int. Cl.**

B22D 23/00 (2006.01)  
B22C 3/00 (2006.01)

(52) **U.S. Cl.** 164/46; 164/24; 164/28; 164/31; 164/32; 164/34; 164/516; 164/72; 106/286.5; 264/643

(58) **Field of Classification Search** 164/46, 164/24, 28, 31, 32, 34, 516, 72, 228, 369, 164/370; 108/286.5; 264/643

See application file for complete search history.

(56) **References Cited**

**U.S. PATENT DOCUMENTS**

7,207,373 B2 \* 4/2007 Parkos et al. 164/369

\* cited by examiner

*Primary Examiner*—Kevin Kerns

*Assistant Examiner*—I.-H. Lin

(74) *Attorney, Agent, or Firm*—Bachman & LaPointe, P.C.

(57) **ABSTRACT**

A substrate is coated by applying an essentially pure aluminum first layer to a surface of the substrate. At least a first portion of the first layer is oxidized so as to provide a protective coating of desired properties. The substrate may be a refractory metal-based investment casting core.

**11 Claims, 2 Drawing Sheets**





FIG. 1



FIG. 2



FIG. 3

## 1

## NON-OXIDIZABLE COATING

CROSS-REFERENCE TO RELATED  
APPLICATION

This is a continuation application of Ser. No. 10/973,132, filed Oct. 26, 2004 and now issued as U.S. Pat. No. 7,207,373, and entitled NON-OXIDIZABLE COATING, the disclosure of which is incorporated by reference herein as if set forth at length.

## BACKGROUND OF THE INVENTION

The invention relates to metallic coating. More particularly, the invention relates to protective coating of oxidizable investment casting cores.

Investment casting is a commonly used technique for forming metallic components having complex geometries, especially hollow components, and is used in the fabrication of superalloy gas turbine engine components.

Gas turbine engines are widely used in aircraft propulsion, electric power generation, and ship propulsion. In gas turbine engine applications, efficiency is a prime objective. Improved gas turbine engine efficiency can be obtained by operating at higher temperatures, however current operating temperatures in the turbine section exceed the melting points of the superalloy materials used in turbine components. Consequently, it is a general practice to provide air cooling. Cooling is provided by flowing relatively cool air from the compressor section of the engine through passages in the turbine components to be cooled. Such cooling comes with an associated cost in engine efficiency. Consequently, there is a strong desire to provide enhanced specific cooling, maximizing the amount of cooling benefit obtained from a given amount of cooling air. This may be obtained by the use of fine, precisely located, cooling passageway sections.

A well developed field exists regarding the investment casting of internally-cooled turbine engine parts such as blades and vanes. In an exemplary process, a mold is prepared having one or more mold cavities, each having a shape generally corresponding to the part to be cast. An exemplary process for preparing the mold involves the use of one or more wax patterns of the part. The patterns are formed by molding wax over ceramic cores generally corresponding to positives of the cooling passages within the parts. In a shelling process, a ceramic shell is formed around one or more such patterns in well known fashion. The wax may be removed such as by melting in an autoclave. The shell may be fired to harden the shell. This leaves a mold comprising the shell having one or more part-defining compartments which, in turn, contain the ceramic core(s) defining the cooling passages. Molten alloy may then be introduced to the mold to cast the part(s). Upon cooling and solidifying of the alloy, the shell and core may be mechanically and/or chemically removed from the molded part(s). The part(s) can then be machined and treated in one or more stages.

The ceramic cores themselves may be formed by molding a mixture of ceramic powder and binder material by injecting the mixture into hardened steel dies. After removal from the dies, the green cores are thermally post-processed to remove the binder and fired to sinter the ceramic powder together. The trend toward finer cooling features has taxed core manufacturing techniques. The fine features may be difficult to manufacture and/or, once manufactured, may prove fragile. Commonly-assigned co-pending U.S. Pat. No. 6,637,500 of Shah et al. discloses general use of refractory

## 2

metal cores in investment casting among other things. Various refractory metals, however, tend to oxidize at higher temperatures, e.g., in the vicinity of the temperatures used to fire the shell and the temperatures of the molten superalloys. Thus, the shell firing may substantially degrade the refractory metal cores and, thereby produce potentially unsatisfactory part internal features. Use of protective coatings on refractory metal core substrates may be necessary to protect the substrates from oxidation at high temperatures. An exemplary coating involves first applying a layer of chromium to the substrate and then applying a layer of aluminum oxide to the chromium layer (e.g., by chemical vapor deposition (CVD) techniques). However, particular environmental/toxicity concerns attend the use of chromium. Accordingly, there remains room for further improvement in such coatings and their application techniques.

## SUMMARY OF THE INVENTION

One aspect of the invention involves an investment casting core having a refractory metal-based substrate and an essentially chromium-free coating directly atop the substrate. The coating includes a first layer consisting principally of aluminum oxide. The first layer has a first thickness in excess of 2.0 $\mu$ . Optionally, a base layer may be located atop the substrate and consist principally of non-oxidized aluminum. Optionally, a transition layer may be located between the first layer and the base layer.

In various implementations, the substrate may be molybdenum-based. The first layer may consist essentially of aluminum oxide and the first thickness may be a nominal (e.g., a median) first thickness. The first thickness may be at least 4.0 $\mu$ . A combined thickness for the base layer and transition layer, if either or both are present, may be no more than the first thickness. The core may be a first core in combination with a ceramic second core and a hydrocarbon-based material in which the first core and the second core are at least partially embedded.

Another aspect of the invention involves a method for coating a substrate. An essentially pure aluminum initial layer is applied to a surface of the substrate. At least a first portion of the initial layer is oxidized so as to leave the first portion with an unoxidized aluminum content of no more than 10% of a total aluminum content and a thickness of at least 2.0 $\mu$ .

In various implementations, the applying may form the initial layer with a characteristic thickness of about 25 $\mu$ -75 $\mu$ . The applying may include at least one of ion vapor deposition, cold spray, and electrolytic deposition. The applying may consist essentially of ion vapor deposition. The oxidizing may include at least one of anodizing, hard coating, and micro-arc oxidation. The substrate may include at least one of a refractory metal-based material, an aluminum alloy, and a non-metallic composite. The substrate may consist essentially of a molybdenum-based material. The oxidizing may oxidize a majority of the aluminum in the applied initial layer. The method may be used to form an investment casting core component.

The method may further include assembling the core with a second core. A sacrificial material may be molded to the core and second core. A shell may be applied to the sacrificial material. The sacrificial material may be essentially removed. The metallic material may be cast at least partially in place of the sacrificial material. The core, second core, and shell may be destructively removed. Alternatively, the second core may be formed at least partially over the core.

Another aspect of the invention involves an article having a substrate having an essentially chromium-free surface. An essentially chromium-free coating is located directly atop the surface. The coating includes a first layer consisting essentially of aluminum oxide. The first layer has a first thickness in excess of about  $2.0\mu$ . Optionally, a base layer may be located directly atop the surface and consist essentially of non-oxidized aluminum. Optionally, a transition layer may be located between the first layer and the base layer.

In various implementations, the substrate may be molybdenum-based. The first layer may the first layer may have a density of at least 3.4 g/cc and a principally  $\alpha$ -phase microstructure. The first layer may have a density of 3.6-4.0 g/cc and an essentially  $\alpha$ -phase microstructure.

The details of one or more embodiments of the invention are set forth in the accompanying drawings and the description below. Other features, objects, and advantages of the invention will be apparent from the description and drawings, and from the claims.

#### BRIEF DESCRIPTION OF THE DRAWINGS

FIG. 1 is a cross-sectional view of a shelled investment casting pattern for forming a gas turbine engine airfoil element.

FIG. 2 is a sectional view of a refractory metal core of the pattern of FIG. 1.

FIG. 3 is a flowchart of processes for forming and using the pattern of FIG. 1.

Like reference numbers and designations in the various drawings indicate like elements.

#### DETAILED DESCRIPTION

FIG. 1 shows a shelled investment casting pattern 20 including a pattern 22 and a ceramic shell 24. The pattern 22 includes a sacrificial wax-like material 26 (e.g., natural or synthetic wax or other hydrocarbon-based material) at least partially molded over a core assembly. The core assembly includes a ceramic feed core 28 having a series of generally parallel legs 30, 32, and 34 for forming a series of generally parallel, spanwise-extending, feed passageways in the ultimate part being cast (e.g., a gas turbine engine turbine blade, or vane). Assembled to the feed core 28 are a series of refractory metal cores (RMCs) 36 and 38. Portions of the RMCs 36 and 38 may be received in compartments 40 and 42 in the feed core 28 and secured therein via ceramic adhesive 44. Other portions of the RMCs 36 and 38 may be embedded in the shell 24 so that the RMCs 36 and 38 ultimately form outlet passageways from the feed passageways to the exterior surface of the part. The exemplary RMCs 36 provide film cooling passageways for airfoil pressure and suction side surfaces and the exemplary RMC 38 provides airfoil trailing edge cooling. Many other configurations are possible either in the prior art or yet to be developed.

FIG. 2 shows further details of one of the RMCs (e.g., 38). The exemplary RMC 38 has a substrate 50 of refractory metal or a refractory metal-based alloy, intermetallic, or other material. Exemplary refractory metals are Mo, Nb, Ta, and W. These may be obtained as wire or sheet stock and cut and shaped as appropriate. A coating system includes an aluminum first layer 52 atop the substrate and an aluminum oxide (alumina) second layer 54 atop the first layer 52. It is believed that  $\alpha$ -phase alumina offers advantageous hardness and adhesion/retention over a broad temperature range.

Nevertheless other phases (e.g., material comprising or consisting essentially of one or both of  $\beta$ - and  $\gamma$ -phase) may be used. Exemplary alumina density is 3.4-4.0 g/cc

The exemplary substrate 50 is formed, e.g., from sheet stock having a surface including a pair of opposed faces 56 and 58 with a thickness T between. Complex cooling features may be stamped, cut, or otherwise provided in the substrate 50. An interior surface 60 of the coating system and first layer 52 sits atop the exterior surface of the substrate 50 and an exterior surface 62 of the coating system and second layer 54 provides an exterior surface of the RMC 38. A transition 64 separates the first layer 52 from the second layer 54. The transition 64 may be fairly abrupt or may be a transition region characterized by a compositional median or compositional gradation. In the exemplary embodiment, the coating system has a thickness  $T_1$ , the first layer 52 has a thickness  $T_2$ , and the second layer 54 has a thickness  $T_3$ .

FIG. 3 shows an exemplary process 200 of manufacture and use (simplified for illustration). The substrate(s) are formed 202 such as via stamping from sheet stock followed by subsequent bending or other forming to provide a relatively convoluted shape for casting the desired features. An essentially pure aluminum coating is deposited 204 atop the substrate. The deposition process may be a physical or chemical deposition process. Exemplary physical deposition processes are ion vapor deposition (IVD) and cold spray deposition. Exemplary IVD and cold spray deposition techniques are shown in U.S. Military Standard Mil-C-83488 (for pure Al) and U.S. Pat. No. 5,302,414 of Alkhimov et al., respectively. Exemplary chemical processes include electrolytic plating. The deposited aluminum layer is then at least partially oxidized 206 to form the second layer 54 and leave the first layer 52. Exemplary oxidation is via chemical process such as anodizing, hard coating (a family of high voltage anodizing processes), and micro-arc oxidation. Exemplary micro-arc processes are shown in U.S. Pat. Nos. 6,365,028, 6,197,178, and 5,616,229.

The RMCs are then assembled to the feed core(s) which may be formed separately 210 (e.g., by molding from silicon-based material) or formed as part of the assembling (e.g., by molding the feed core partially over the RMCs). The assembling may also occur in the assembling of a die for overmolding 212 the core assembly with the wax-like material 26. The overmolding 212 forms a pattern which is then shelled 214 (e.g., via a multi-stage stuccoing process forming a silica-based shell). The wax-like material 26 is removed 216 (e.g., via steam autoclave). After any additional mold preparation (e.g., trimming, firing, assembling), a casting process 218 introduces one or more molten metals and allows such metals to solidify. The shell is then removed 220 (e.g., via mechanical means). The core assembly is then removed 222 (e.g., via chemical means). The as-cast casting may then be machined 224 and subject to further treatment 226 (e.g., mechanical treatments, heat treatments, chemical treatments, and coating treatments).

The coating process may provide an initial aluminum thickness in the range of 0.25-5 mil ( $6-130\mu$ ), more preferably 1-3 mil ( $25-75\mu$ ). Some of this material is then oxidized to form the second layer 54. During the oxidation, some of the aluminum may be lost (e.g., into the anodizing bath). Advantageously, little if any of the aluminum diffuses into the substrate at least until firing/casting. At those elevated temperatures, some or all of the theretofore unoxidized aluminum may diffuse into/with the substrate material. The oxidation may advantageously form the second layer with the thickness  $T_3$  in the vicinity of  $5\mu$  or more to provide

adequate insulation. More broadly, the thickness may be in excess of  $2\mu$  (e.g.,  $4\mu$ - $50\mu$ , or  $20$ - $40\mu$ ). Advantageously, at least 90% of the aluminum in the second layer 54 may be oxidized. The oxidation tends to expand the thickness of the second layer by 100% relative to the thickness of the deposited aluminum being oxidized. Thus, in the absence of diffusion or loss, a  $25\mu$  deposited aluminum layer could, if oxidized across its thickness, produce an aluminum oxide layer of thickness in the vicinity of  $50\mu$ . With a 20% loss and oxidation across substantially half the depth, the remaining first layer thickness  $T_2$  would be about  $10\mu$  and the aluminum oxide second layer thickness  $T_3$  would be about  $20\mu$ . The foregoing numbers are merely exemplary.

Advantageously, however, at least with the exemplary molybdenum substrate and various anodization processes, the first layer thickness is at least about  $2.0\mu$ . That is the minimum thickness believed appropriate to isolate the substrate from the effects of the anodization. If the thickness  $T_2$  becomes less, the molybdenum may begin to dissolve, destroying the coating adherence. There is no inherent upper limit to the thickness  $T_2$ . However, excess thickness poses cost issues and represents a loss of insulation contrasted with the situation where such excess material is converted to alumina. Thus, typically, the alumina thickness  $T_3$  will be at least half the total coating thickness  $T_1$ .

The coating technique may have broader applicability. For example, the substrate may be of highly alloyed aluminum atop which the purer aluminum layer is deposited and then at least partially oxidized. Alternatively, the substrate may be a composite material.

Various dopants or alloying elements may be used. Ca, Mg, Si, and Zr, for example, form stable oxide systems  $\text{CaO}$ ,  $\text{MgO}$ ,  $\text{SiO}_2$ ,  $\text{ZrO}_2$ . These elements or their combinations may be deposited in an alloy with the aluminum to be oxidized (e.g., in exemplary low quantities of less than 1% by weight to control grain growth and the morphology of the coating and influence properties such as CTE). Greater quantities of these elements (including even major portions of the as-applied coating—pre-oxidation) are possible.

The present system and methods may have one or more advantages over chromium-containing coatings. Notable is reduced toxicity. Chromium containing coatings are typically applied using solutions of hexavalent chromium, a particularly toxic ion. Furthermore, when the coated core is ultimately dissolved, some portion of the chromium will return to this toxic valency. The present coatings may have less than 0.2%, preferably less than 0.01% chromium by weight, and, most preferably, no detectable chromium. The present system and methods may have one or more advantages over single-step coating of a substrate (e.g., molybdenum) with aluminum oxide. The aluminum oxide layer may have higher density. A greater evenness may be obtainable by using aluminum deposition techniques that do not suffer from the same line-of-sight problems as various single-step aluminum oxide deposition techniques.

One or more embodiments of the present invention have been described. Nevertheless, it will be understood that various modifications may be made without departing from the spirit and scope of the invention. For example, the coatings may be utilized in the manufacture of cores of existing or yet-developed configuration. The details of any such configuration may influence the details of any particular implementation as may the details of the particular ceramic core and shell materials and casting material and

conditions. Accordingly, other embodiments are within the scope of the following claims.

What is claimed is:

1. A method for coating a substrate for forming a casting core comprising:
  - applying an essentially pure aluminum initial layer to a surface of the substrate; and
  - oxidizing at least a first portion of the initial layer so as to leave the first portion with an unoxidized aluminum content of no more than 10% of a total aluminum content and a thickness of the first portion of at least  $2.0\mu$ .
2. The method of claim 1 wherein the applying forms the initial layer with a characteristic thickness of  $25\mu$ - $75\mu$ .
3. The method of claim 1 wherein the applying comprises at least one of:
  - ion vapor deposition;
  - cold spray; and
  - electrolytic deposition.
4. The method of claim 1 wherein the applying consists essentially of ion vapor deposition.
5. The method of claim 1 wherein the oxidizing comprises at least one of:
  - anodizing;
  - hard coating; and
  - micro-arc oxidation.
6. The method of claim 1 wherein the substrate comprises at least one of:
  - a refractory metal-based material;
  - an aluminum alloy; and
  - a non-metallic composite.
7. The method of claim 1 wherein the substrate consists essentially of:
  - a molybdenum-based material.
8. The method of claim 1 wherein the oxidizing oxidizes a majority of the aluminum in said applied initial layer.
9. The method of claim 1 wherein the first portion has a density of at least  $3.4\text{ g/cc}$  and a principally  $\alpha$ -phase microstructure.
10. The method of claim 1 wherein the core is a first core and the method further comprises:
  - assembling the first core with a second core;
  - molding a sacrificial material to the first core and the second core;
  - applying a shell to the sacrificial material;
  - essentially removing the sacrificial material;
  - casting a metallic material at least partially in place of the sacrificial material; and
  - destructively removing the first core, the second core, and the shell.
11. The method of claim 1 wherein the core is a first core and the method further comprises:
  - forming a second core partially over the first core;
  - molding a sacrificial material to the first core and the second core;
  - applying a ceramic shell to the sacrificial material;
  - essentially removing the sacrificial material;
  - casting a metallic material at least partially in place of the sacrificial material; and
  - destructively removing the first core, the second core, and the shell.